

C. H. SHEASLEY.  
LUBRICATING CAKE AND METHOD OF MAKING SAME.  
APPLICATION FILED JAN. 22, 1916.

1,180,547.

Patented Apr. 25, 1916.

Fig. 1.



Fig. 2.



Fig. 3.



Fig. 4.



Charles H. Sheasley Inventor

By  
Maxine Cameron Lewis & MacLean  
Attorneys

# UNITED STATES PATENT OFFICE.

CHARLES H. SHEASLEY, OF FRANKLIN, PENNSYLVANIA.

## LUBRICATING-CAKE AND METHOD OF MAKING SAME.

1,180,547.

Specification of Letters Patent. Patented Apr. 25, 1916.

Application filed January 22, 1916. Serial No. 73,650.

To all whom it may concern:

Be it known that I, CHARLES H. SHEASLEY, a citizen of the United States of America, and a resident of Franklin, Pennsylvania, have invented a new and useful Improvement in Lubricating-Cakes and Methods of Making Same, which invention is fully set forth in the following specification.

This invention relates to the art of lubrication, and more particularly to lubricants designed to be employed in a solid form. When solid lubricants are employed, it is desirable in many of the conditions of use, to mold the lubricant into the form of the lubricating box or other container in which it is to be placed for use, in order to facilitate the ready application of the lubricant. Furthermore, the lubricant must be hard in order that it may withstand high pressures and temperatures without undue wear or waste. As an example, it is customary in applying solid lubricants to the journals of locomotive engines to employ a lubricating box in which is placed a solid cake of the lubricant previously molded to the form of the box and having a concave surface which is placed adjacent to the journal. The lubricant is applied to the journal by pressure. An example of an axle box lubricator of this type is shown and described in U. S. Letters-Patent No. 818,022, dated April 17, 1906.

It has heretofore been the practice to ship the solid lubricant in large masses packed in barrels or other containers. When it is desired for use, it is either taken cold and forced into a suitable mold for giving it the desired shape, or it is remelted and cast into a mold of the proper form for this purpose. Each of these methods of molding the lubricant is open to serious objection, inasmuch as they materially change the proportions of the ingredients of which the lubricant is composed, to the detriment of its lubricating qualities, and also change the structure and general physical characteristics of the lubricant, also to the serious detriment of its lubricating qualities. It is desirable that lubricants employed for this purpose shall contain as large an amount of mineral oil as possible. At the same time the lubricant must be hard in order to be durable and to retain the form in which it is to be applied. This has been accomplished heretofore by incorporating the mineral oil

with ingredients suitable for making hard soap as, for example, tallow treated with an alkali sufficient to convert the fat into a hard soap and leave the alkali in excess, the alkali being introduced in the form of an alkali solution. When an attempt is made to press this lubricant into the desired form in a cold state, it is found that the pressure necessary to impart the form to the lubricant causes an exudation of water, glycerin and alkali solution therefrom. This causes a deterioration in its lubricating qualities, since the water, the glycerin, and the alkali solution each performs a desirable function in the lubricating body. Moreover, this cold molding produces a material change in the structure of the lubricant. It is irregular and granular in structure, quite soft, and easily broken. The surface of the cold molded lubricant is soft, and moisture, glycerin and the alkali solution continue to exude therefrom after the molding operation is completed. In a short time after the molding operation, the alkali effloresces in spots on the surface as a solid incrustation which is detrimental to its lubricating qualities. Moreover, the liquid exudations cause a sticky, damp condition on the surface of the cake of lubricant which injures a pasteboard or paper packing case, renders it difficult to handle, and causes cinders and dirt to adhere thereto. The sum total of the results obtained by cold molding is an inferior lubricant, due to its change in physical characteristics; the parting with moisture, glycerin, and alkali solution during the pressing operation; the continued parting with these substances after the molding operation; and the incrustation of alkali upon the surface. And its durability and lubricating qualities are decreased by reason of its softness and changed structural condition.

If an attempt be made to mold the lubricant by remelting after it is once made and permitted to cool, that is, if it be taken from the container in which it was originally placed at the time of manufacture, remelted and then cast into a mold, it has been found that the remelting requires a temperature far exceeding that required to prepare the original composition, and approximating in fact from 425° to 450° F. This high remelting temperature necessarily results in driving off a very large part of the moisture contained in the lubricant, and, upon pour-

ing the mass into a mold and allowing it to cool therein, it assumes a fine spongy condition, is soft, easily indented by the pressure of the finger, and very light. It is easily broken, dry, and granular. The high temperature required to melt the lubricant causes considerable decomposition, with the evolution of moisture and the pungent odor of acrolein, indicating the decomposition of the constituents. And the high temperature of melting almost completely destroys the lubricating qualities of the substance. These difficulties, experienced when attempts are made to remelt and mold the lubricant, are so serious that they have practically prohibited the employment of the lubricant in this way, and have greatly handicapped its use by cold molding.

The object of the present invention is to provide a hard lubricant molded into suitable form for use in a lubricant container, and which shall be free from the aforementioned objections.

With this object in view, the invention consists in a molded cake of lubricant and the process of manufacturing the same. The particular form in which the lubricant is molded will be governed by the form of the lubricant container or lubricant cellar in which it is designed to be used. In some cases, as for example, that shown in Patent No. 818,022 above referred to, the lubricant cellar is provided with a perforated concave top and a flat, spring-pressed follower, and the molded cake for use in such cellar should have a form in horizontal cross-section approximating that of the cellar or lubricant container. The top of the molded cake of lubricant may be either provided with a cavity corresponding to the surface to be lubricated, with the opposite side flat, or the molded block of lubricant may have a flat top and a flat bottom. In either case the molded block of lubricant is pressed against the journal to be lubricated by the follower in the lubricant container.

I have discovered that if mineral oil be mixed with hard soap stock, such as tallow, or the derivatives thereof capable of being converted into hard soap, and the mixture then treated with a suitable caustic alkali, as caustic soda, for saponifying the hard soap stock, the alkali being in excess, and the product cast into a suitable mold before the reaction of saponification is complete, there will result a hard, tough, durable, homogeneous molded cake of lubricant possessing the maximum of efficiency as a lubricant, and from which neither moisture, glycerin, nor alkali will exude; and which, in short, will supply a highly efficient, durable lubricant in convenient form ready for use, and which will eliminate all of the objections hereinbefore described. When made according to my invention, the molded cake

has an extremely firm or case-hardened surface, which acts to prevent the exudations mentioned above, and also materially assists in preventing the drying out of the cake while in storage before use.

My invention will be best understood by reference to the accompanying drawings, in which—

Figure 1 is a vertical cross-sectional perspective of a mold in which the lubricant is cast, showing the lubricant therein; Fig. 2 is a perspective view of the molded cake after it is taken out of the mold of Fig. 1; Fig. 3 is a cross-sectional view of a journal and the lubricating cellar or container thereof, with the cake of lubricant in position therein; and Fig. 4 is a perspective view of a molded cake of lubricant having a flat top and bottom.

In the practice of the invention, I take mineral oil and any suitable hard soap stock (such, for example, as tallow or the fatty acids thereof capable of being employed in the manufacture of hard soap), and thoroughly mix the same under a temperature which will facilitate incorporation of the oil with the stock. I have found a temperature of 115° to 125° F. to serve this purpose. The proportions of the soap stock and mineral oil employed will depend upon the structural characteristics desired in the lubricant. After the mineral oil and the soap stock have been thoroughly mixed, I permit the temperature to fall to approximately 105° F., and then treat the mass with an alkali to convert the soap stock employed into a hard soap, the alkali, such for example as caustic soda, being preferably introduced in the form of a solution composed of equal parts by weight of caustic soda and water, the quantity of the alkali solution employed being in excess, and preferably 50% in excess, of the chemical equivalent of the soap stock used. Most excellent results are obtained by employment of the following proportions of ingredients by weight, to wit:

|                  |          |
|------------------|----------|
| Tallow-----      | 14. lbs. |
| Mineral oil----- | 9.7 lbs. |
| Soda lye-----    | 3. lbs.  |
| Water-----       | 3. lbs.  |

The alkali solution is introduced at approximately a temperature of 105° F., and preferably it is sprayed into the mixture. The entire mass is agitated during the spraying operation, and as soon as the alkali solution is sprayed into the mixture and thoroughly incorporated therewith, and before the reaction of saponification is complete, I pour the mixture into a suitable mold, and permit the reaction of saponification to be carried to completion while the mass is within the mold. The chemical reaction will cause a very marked rise in the temperature of the mass. This temperature

will be found to be from 175° to 250° F., depending upon the quantities of the materials employed.

Referring to Fig. 1, 1 is a mold which preferably is of pasteboard or fiber, since when such a mold is employed, the removal of the cast cake of lubricant therefrom is greatly facilitated; and 2 is the cake of lubricant therein. After the mass is poured into the mold 1, the mold is preferably covered by any suitable cover, as for example, the cover 3 shown in dotted lines in Fig. 1. The mold is provided with a convex bottom 4, and when the molded cake of lubricant 5 is removed from the mold, it will have the form shown in Fig. 2. If, however, the same be cast in a mold having a flat bottom, it will have the form of the cake 6, shown in Fig. 4.

When the lubricant container is in the form of the lubricant cellar 7, shown in Fig. 3, said cellar is sometimes, though not necessarily, provided with a perforated cap portion 8 having a concave upper surface conforming to the cylindrical outline of the journal 9. Preferably, cake 5 of Fig. 2 is used in this form of lubricant container, the same being supported upon the follower 10 pressed upward by the spring 11. When such cake has been largely consumed so as to leave only the upper concave portion unconsumed, it may be either removed and another similar cake inserted in its place, or the flat cake 6 of Fig. 4 may be placed under the unconsumed portion of the lubricant cake in the cellar without removing the same, thus effecting the economical consumption of all of the lubricant. If desired, the flat cake 6 might be employed in the first instance, and the concavity worn therein as the cake is consumed, but as indicated above, I prefer to start the operation with the cake 5 of Fig. 2.

It will be apparent that if the lubricant were molded into a cake say double the length desired for use in the lubricant container, and then cut in two to form two cakes of equal size, it would still be within the spirit of my invention, though the surface where the cut occurred would not be a case-hardened surface, and I therefore prefer to cast the lubricant in the form of single cakes ready for use. Nevertheless, I desire it distinctly understood that a cake molded to form by pouring the lubricant into a mold during the reaction of saponification, and then cut into proper lengths suitable for use in a lubricant container would be within the purview of my invention.

The matter of maintaining the lubricant with its original physical structure which it assumes when saponification is complete, is of the highest importance. When this is done, the lubricating qualities of the lubri-

cant are superior to any results obtained when the lubricant is cold molded under pressure, and the durability of the lubricant is increased by approximately 50%. As indicated above, if the lubricant is remelted and then molded, its lubricating properties are practically destroyed.

When a lubricant is made in accordance with my invention, it retains all of the moisture originally introduced therein and the product of saponification, whether glycerin or water, resulting from the chemical reaction of the alkali on the soap stock, and the excess alkali is uniformly distributed throughout the mass and emulsifies the mineral oil. Moreover, the molded cake of lubricant will be found to have a glazed or case-hardened surface, which effectually occludes the moisture, the glycerin and the alkali within the cake, thereby preventing the loss of the moisture by evaporation, and exudation of the glycerin and alkali, and consequent efflorescence of the latter. The mass of the lubricant is of a uniform and homogeneous texture, non-granular, tough and hard. These properties materially contribute to the efficiency of the mass as a lubricant, and to its lasting and wearing properties, thus making not only for effectiveness in lubrication, but economy in use. Its durability results from its compact and uniform structure and the retention of its constituents in their original proportions and its adaptability to the incorporation of a large quantity of mineral oil, while still retaining its structural form.

From the foregoing, it will be perceived that I have provided a lubricant molded into suitable form for use in the lubricant container, and in which the proportions and the constituents of the original lubricant are retained in the molded cake; and which employs a large amount of mineral oil, recognized as desirable in such lubricants, and which is hard in texture, tough and durable. So far as I am informed, this has never before been accomplished.

It will be understood by those skilled in the art that the proportions of ingredients and the temperatures herein indicated may be varied within limits, and such proportions and temperatures are herein given for the purpose of clearly describing the invention, and not for the purpose of defining the limits thereof, reference being had to the claims for this purpose.

What is claimed is:

1. The process of making a lubricant cake for a lubricant container consisting in mixing hard soap stock, mineral oil and excess of alkali solution, then pouring the mixture into a lubricant cake mold to saponify and solidify therein.

2. The method of making a solid lubricant cake for use in lubricant containers,

which consists in mixing together mineral oil, hard soap stock and an alkali solution, the alkali being in excess, and then molding the mass into suitable form for use in a lubricant container during the reaction of saponification.

3. The method of making a solid lubricant cake for use in lubricant containers, which consists in mixing together in the presence of heat mineral oil, hard soap stock and an alkali solution, the alkali being in excess, and then casting the mass into suitable form for use in a lubricant container before the reaction of saponification is complete.

4. The method of making a lubricant cake for a lubricant container, which consists in mixing mineral oil and hard soap stock at a temperature of approximately 125° F., then lowering the temperature to approximately 105° F., then introducing alkali in solution at approximately 105° F., the alkali being in excess of the amount necessary to saponify the soap stock, and then before the reaction of saponification is complete pouring the mass into a mold having the form of the container.

5. The method of making a lubricant cake for a lubricant container, consisting in mixing hard soap stock and mineral oil at a temperature of approximately 125° F., then lowering the temperature to approximately 105° F., then introducing alkali in solution at approximately 105° F., the alkali being in excess of the amount necessary to saponify the soap stock whereby the temperature of the mass will be raised as the result of the reaction, and then before the reaction of saponification is complete pouring the mass into a mold having the form of the container.

6. The method of making a lubricant cake for a lubricant container, which consists in mixing mineral oil and a hard soap stock in the presence of heat, then introducing alkali in solution into the mass, and then before the reaction of saponification is complete pouring the mass into a mold having the form of the container.

50 7. A cast cake of lubricant for use in a lubricant container, said cake consisting of mineral oil, soap associated with the product of its saponification and an alkali solution, the same being cast direct from the fluid state of its original manufacture into suitable form for use in said container.

8. A cast cake of lubricant for use in a lubricant container, said cake consisting of mineral oil, soap associated with the product of its saponification and an alkali solution, the same being cast during the saponifying reaction of its manufacture into suitable form for insertion in said container.

60 9. A cast cake of lubricant for use in a

lubricant container, said cake containing mineral oil, hard soap and free alkali, the same being cast during the saponifying reaction of its manufacture into suitable form for insertion in said container.

10. A cast cake of lubricant for use in a lubricant container, said cake containing mineral oil and hard soap and being cast during the saponifying reaction of its manufacture into suitable form for insertion in said container.

75 11. A case-hardened cast cake of lubricant for use in a lubricant container, said cake containing mineral oil, hard soap and free alkali, the same being cast during the saponifying reaction of its manufacture into suitable form for insertion in said container.

12. A cast cake of lubricant for use in a lubricant container and having a form to fit the lubricant container, said cake containing mineral oil, hard soap and free alkali and having the physical characteristics resulting from the saponifying reaction.

13. A cast lubricant for use in a lubricant container and having a form to fit the lubricant container, said cake containing mineral oil and hard soap and having the molecular arrangement assumed on solidifying at the close of the saponifying reaction.

95 14. A cast cake of lubricant for use in a lubricant container, said cake consisting of mineral oil, soap associated with the glycerin of saponification, and an alkali solution, the same being cast during the saponifying reaction of its manufacture into suitable form for insertion in said container.

15. A case-hardened cast cake of lubricant for use in the lubricant container of a locomotive or the like, said cake containing mineral oil, hard soap and free alkali and having a form to fit the lubricant container.

110 16. A case-hardened cast cake of lubricant for use in the lubricant container of a locomotive or the like, said cake consisting of mineral oil, hard soap associated with the glycerin of saponification and an alkali solution and having a form to fit the lubricant container.

115 17. A cast cake of lubricant for use in a lubricant container and having a form to fit the lubricant container, said cake being of a dense uniform structure throughout its mass and consisting of mineral oil, soap associated with the product of its saponification and an alkali solution.

120 18. A cast cake of lubricant for use in a lubricant container and having a form to fit the lubricant container, said cake consisting of mineral oil, soap associated with the product of its saponification and an al-

kali solution and having all the physical characteristics resulting from the saponifying reaction.

19. A cast cake of lubricant for use in a lubricant container, said cake containing mineral oil, soap associated with the product of saponification and an alkali solution, said elements having the relative molecular arrangement assumed on solidifying at the 10 close of the saponifying reaction.

20. A cast cake of lubricant for use in a lubricant container, said cake containing mineral oil, hard soap associated with the glycerin of saponification and an alkali solution, said elements having the relative 15 molecular arrangement assumed on solidifying at the close of the saponifying reaction.

In testimony whereof I have signed this specification.

CHARLES H. SHEASLEY.